# EUROPEAN PATENT SPECIFICATION

(11) **EP 0 896 800 B1**
(45) Date of publication and mention of the grant of the patent: **05.02.2003**
(21) Application number: 98114141.9
(22) Date of filing: 29.07.1998
(51) Int. Cl.: A41D 19/015

(54) **Sailing glove and line combination**
Kombination eines Segelhandschuhs und einer Leine
Gant de navigation et cordage combinés

(30) Priority: 11.08.1997 US 908047
(43) Date of publication of application: 17.02.1999
(73) Proprietor: Harken, Inc., Pewaukee, Wisconsin 53072 (CH)
(72) Inventor: Harken, Olaf T., Pewaukee, WI 53072 (US); Gravengood, Charles E., Glenview, IL 60025 (US)
(74) Representative: Flosdorff, Jürgen, Dr.

(56) References cited:
- EP-A- 0 482 618
- FR-A- 2 656 597
- US-A- 4 497 072
- US-A- 5 117 509
- US-A- 5 511 248
- US-A- 5 625 900

## Description

### Background of the Invention

This invention relates a sailing glove for handling lines on sailing vessels.

Sailing gloves have been traditionally constructed of leather, with reinforcing pads on the palms and fingers. These gloves tend to become stiff after repeated wetting and drying. Thick, heavy leather is employed, since soft leather tends to wear out quickly.

More recently, artificial leather has been used as a component in sailing gloves. Artificial leather is typically composed of microfine polymer fibers such as nylon, with the fibers being interfelted by mechanical entanglement such as by needling, with the resultant nonwoven being impregnated with a cured polyurethane resin to bond the fibers together. These gloves have about the same gripping power and wear rate of natural leather but also have the added benefit of remaining soft after being wetted and dried.

Recent advances in sailing products have led to advances in technology relating to the lines or sheets which control the sails. For example, lines are made from high tensile polymer strands having low elongation, and allow for a smaller diameter line to be used. These lines also tend to have a slippery surface, making them difficult to grip and control.

Heretofore, sailing gloves have had only a single purpose, and that is to prevent chafing of the skin of the palm and fingers of the hand. The ability to hold a line against an opposing force, such as the sheet of a sail, has been determined solely by the strength and endurance of the sailor. In many cases, sheets are held by hand, rather than cleated, to enable quick sail adjustments, and fatigue becomes an important factor especially in cold conditions.

US-A-5 625 900 discloses a glove for cold weather which is especially useful in skiing and the like. The glove comprises surfaces for gripping which comprise a porous substrate of nonwoven fibres and a layer of a tackifying resin consisting of Silicone being applied to the porous substrate.

### Summary of the Invention

In accordance with the present invention, the gripping surfaces of a sailing glove are provided with a high coeficient of friction relative to the sailing line. Specifically, the gripping surfaces are tackified to provide a coefficient of friction of from about 0.6 to about 0.9 relative to the line. Surprisingly, this has been found to increase the gripping power of the sailor and glove up to 50 % over untreated gloves without affecting the ability to smoothly release and regrip the line.

The exposed palm and finger portions of the sailing glove are composed of porous artificial leather which has been treated or impregnated with a tackifying agent, such as a short chain polyurethane or tackifying resin. The material remains soft after repeated wet and dry cycles, and the wear properties are approximately the same as an untreated artificial leather.

### Brief Description of the Drawings

Figure 1 is a plan view of the sailing glove of the present invention, shown in connection with a section of line.

### Description of the Preferred Embodiments.

Figure 1 illustrates the palm side of a sailing glove 10 in combination with a line 12 to be grasped when the glove is used. The forces on the line act generally in the direction indicated by the arrow 14, namely, perpendicular to or across the palm and fingers.

As used herein, the term "line" means a intertwined or braided and flexible rope-like structure composed of polymeric strands, such as polyester, aramid, polyamid or polyolefin polymers, sometimes having an outer textile cover. Lines on sailing craft are normally used to control the trim of sails or the rigging.

The palm 16, thumb 17, and inner finger portions 18 of the glove are lined with a thin layer of artificial leather 19 as shown, held to the fabric of the glove by stitching, such as that shown at 20, or by other type of bonding. As is typical of many sailing gloves, the ends of the finger portion of the glove may be cut away as shown at 22.

Artificial leather is a commercially available material sold under the trademark Amara. Preferably, porous types of artificial leather are employed. Such materials are made from a nonwoven substrate of short microfine nylon or other polymer fibers which are formed into a web by carding and cross lapping. The web is then needled with barbed needles at a high rate to entangle the fibers. The fabric is then impregnated with a polyurethane resin and the resin is coagulated. Various techniques are employed to provide a porous surface, such as application of a solvent, as described in U.S. patent no. 5,156,900.

A short chain polyurethane tackifying resin or polymer or agent is incorporated into the artificial leather at a rate of five to twenty percent of the weight of the substrate. The agent may be dissolved in a solvent for this purpose. The actual amount of tackifying agent employed depends on the nature of the agent, with the only qualification being that the coefficient of friction between the material and the line 12 must fall within the ranges specified herein.

Both the static and dynamic coefficients can be determined by a simple test using the treated artificial leather from the glove and engaging the material on a support with the line 12. The preferred method is to mount a piece of the treated material on a drum, with the line 12 being looped over the supported material for approximately 180 degrees. The static coefficient of friction is calculated from the maximum force required to start the line moving against various amounts of weights or loads on the line. The dynamic coefficient of friction is calculated by measuring the amount of force required to move the line at a constant speed under increasing amounts of load. Both measurements can be made by inserting a load cell on one side of the drum and applying weight to the other side.

It has been found that the static coefficient of friction between the glove material and the line is critical and must be between 0.6 and 0.9 and the average coefficient should be between about 0.65 and 0.75. The dynamic coefficient between the line and glove material should be in the order of 0.6 to less than 0.9 with the average in the order of between about 0.6 to 0.75. Within these parameters, the glove 10 will provide up to 50% improved gripping power on the line 12, while allowing the line to be easily released and regripped. Artificial leather gloves without a tackifying agent generally have a static coefficient of friction with the line of less than 0.5 and an average dynamic coefficient of less than 0.4.

A variety of other types of materials have been tested, including a number of fabrics having rough surfaces. All other materials proved to be unsatisfactory either because of low gripping power or excessive wear. Despite the higher coefficient of friction afforded by the present glove, the surfaces of the glove in contact with the line exhibit a high wear rate, which is approximately the same as the same untreated artificial leather glove having a lower coefficient of friction with the line. The wear rate from a line can be evaluated by running a line under load back and forth across a 180°expanse of material supported on a stationary drum. Without wishing to be bound by any theory, it is believed that the tackifying resin may serve to protect and reduce wear on the fabric substrate of the artificial leather.

## Claims

1. A sailing line and glove combination, said combination comprising a line having an outer surface of polymer strands, and a glove adapted to grip said line, said glove comprising surfaces for gripping said line, said surfaces comprising a porous substrate of nonwoven fibers, and a tackifying resin applied to said porous substrate
**characterized in that**
said tackifying resin consists of polyurethane,
said substrate is impregnated with said polyurethane,
said surfaces and said line have a static coefficient of friction between 0.6 and 0.9 and
the wear properties of said impregnated substrate are the same as an untreated one.

2. The sailing line and glove combination of claim 1, **characterized in that** the porous substrate of nonwoven fibres is an artificial leather.

3. The sailing line and glove combination of claim 1, **characterized in that** the static coefficient of friction is between 0.65 and 0.75.

4. The sailing line and glove combination of Claim 1 wherein said gripping surfaces and said line have a dynamic coefficient of friction which is smaller than the static coefficient of friction.

## Patentansprüche

1. Kombination eines Segelhandschuhs und einer Leine, wobei die Kombination eine Leine mit einer Außenfläche von Polymerlitzen enthält und der Handschuh geeignet ist, diese Leine zu ergreifen, wobei der Handschuh Flächen zum Greifen der Leine hat, die ein poröses Substrat aus Faserflies enthält und wobei ein klebrigmachendes Harz auf das poröse Substrat aufgebracht ist,
**dadurch gekennzeichnet,**
**daß** das klebrigmachende Harz aus Polyurethan besteht,
**daß** das Subtrat mit dem Polyurethan imprägniert ist,
**daß** die Flächen und die Leine einen statischen Reibungskoeffizienten zwischen 0,6 und 0,9 haben und
**daß** die Abnutzungseigenschaften des imprägnierten Substrats dieselben sind wie bei einem unbehandelten.

2. Kombination eines Segelhandschuhs und einer Leine nach Anspruch 1,
**dadurch gekennzeichnet,**
**daß** das poröse Substrat aus Faserflies ein Kunstleder ist.

3. Kombination eines Segelhandschuhs und einer Leine nach Anspruch 1,
**dadurch gekennzeichnet,**
**daß** der statische Reibungskoeffizient zwischen 0,65 und 0,75 liegt.

4. Kombination eines Segelhandschuhs und einer Leine nach Anspruch 1,
**dadurch gekennzeichnet,**
**daß** die Greifflächen und die Leine einen dynamischen Reibungskoeffizienten haben, der kleiner ist als der statische Reibungkoeffizient.

## Revendications

1. Ensemble de cordage et de gant pour la navigation à voile, ledit ensemble comprenant un cordage comportant une surface externe de torons de polymère, et un gant adapté à la préhension dudit cordage, ledit gant comprenant des surfaces pour saisir ledit cordage, lesdites surfaces comprenant un substrat poreux de fibres non tissées, et une résine donnant du collant appliquée sur ledit substrat poreux **caractérisé en ce que**
ladite résine donnant du collant consiste en polyuréthanne,
ledit substrat est imprégné dudit polyuréthanne,
lesdites surfaces et ledit cordage ont un coefficient de frottement statique entre 0,6 et 0,9, et
les propriétés d'usure dudit substrat imprégné sont les mêmes que celles d'un substrat non traité.

2. Ensemble de cordage et de gant pour la navigation à voile selon la revendication 1, **caractérisé en ce que** le substrat poreux de fibres non tissées est un cuir artificiel.

3. Ensemble de cordage et de gant pour la navigation à voile selon la revendication 1, **caractérisé en ce que** le coefficient de frottement statique est compris entre 0,65 et 0,75.

4. Ensemble de cordage et de gant pour la navigation à voile selon la revendication 1, dans lequel lesdites surfaces de préhension et ledit cordage ont un coefficient de frottement dynamique qui est inférieur au coefficient de frottement statique.
